

Patented Oct. 26, 1926.

1,604,395

# UNITED STATES PATENT OFFICE.

FRED M. EKERT, OF DRESDEN, GERMANY.

## PRODUCTION AND COMPOSITION OF PORCELAIN.

No Drawing. Application filed June 27, 1924, Serial No. 722,713, and in Germany June 28, 1923.

The object of the present invention is a process of producing a difficultly fusible porcelain. There are porcelain masses known consisting of kaolin, clay, silica and feldspar as a flux, but these masses have a relatively low melting point on account of the large proportions of alkalis contained in the feldspar. The present process, however, refers to a method of producing a new porcelain mass possessing increasing resistance to heat. To accomplish this end, I replace the feldspar of the known mixtures by a flux consisting essentially of aluminum fluosilicate. This porcelain being formed to the desired shape, dried and burned.

The chemical formulæ are as follows:

The known mixture consists of clay



and silica =  $\text{SiO}_2$  and



or



According to my invention the feldspar is replaced by a flux consisting essentially of aluminum fluosilicate =  $\text{Al}_2\text{F}_6\text{SiF}_4$ .

These porcelain substances are mixed with water and kneaded into a plastic paste as required in porcelain manufacture. Out of this paste the ware of any desired shape is formed, allowed to dry and then baked in an ordinary porcelain furnace at a temperature of approximately 2370°-2540° Fahrenheit. During the baking process the fluorine, hydrogen (and the hydrocarbon parts of the carbon) evaporate so as to leave only alumina-silica. On account of the absence of alkalis this material possesses a very high melting point exceeding 3300° F. and is therefore far superior to all feldspar-porcelains in resistance to heat and, as insulator, to electric current.

I claim:

The process of producing a difficultly fusible porcelain comprising mixing clay, silica, and a flux consisting essentially of aluminum fluosilicate, and forming to desired shape, drying and burning.

In testimony whereof I have affixed my signature.

FRED M. EKERT.